

## 1

2,772,183

## CHEMICAL NICKEL PLATING PROCESSES

Paul Talmey, Barrington, Ill., and Donald E. Metheny, Hammond, and Warren G. Lee, East Chicago, Ind., assignors to General American Transportation Corporation, Chicago, Ill., a corporation of New York

No Drawing. Application September 24, 1953,  
Serial No. 382,214

21 Claims. (Cl. 117—50)

The present invention relates to improved processes of chemical nickel plating of bodies formed essentially of iron, including the various alloys thereof, i. e. steel, etc., employing baths of the nickel cation-hypophosphite anion type, and more particularly to such processes employing baths of the character disclosed in the copending application of Gregoire Gutzeit, Paul Talmey and Warren G. Lee, Serial No. 376,968, filed August 27, 1953.

The chemical nickel plating of a catalytic material (iron, steel, etc.) employing an aqueous bath of the nickel cation-hypophosphite anion type is based upon the catalytic reduction of nickel cations to metallic nickel and the corresponding oxidation of hypophosphite anions to phosphite anions with the evolution of hydrogen gas at the catalytic surface. The reactions take place when the body of catalytic material is immersed in the plating bath, and the exterior surface of the body is coated with nickel.

In accordance with the process disclosed in the Gutzeit, Talmey and Lee application mentioned, a plating bath is employed that consists essentially of an aqueous solution of a nickel salt and a hypophosphite and a nickel complexing agent and a separate and different exalting additive. The nickel complexing agent is selected from the group consisting of ammonia, amines, acid amines, aminocarbonyls, amine-oxides and polyalcohols, as well as saturated aliphatic hydroxycarboxylic acids, aliphatic aminocarboxylic acids and aliphatic keto acids, and the salts of these compounds. The exalting additive is selected from the group consisting of simple short chain saturated aliphatic dicarboxylic acids and aliphatic aminocarboxylic acids, and the salts of these compounds. In passing it is noted that certain of the nickel complexing agents (ammonia and amines) form molecular complexes with the nickel cations, while the remainder of the nickel complexing agents (hydroxycarboxylic acids, aminocarboxylic acids, etc.) form inner complexes or chelates with the nickel cations.

These plating baths are particularly advantageous in carrying out the chemical nickel plating process in that they exhibit very fast plating rates, and accommodate the utilization thereof in a continuous system of the character of that disclosed in the copending application of Paul Talmey and William J. Crehan, Serial No. 222,222, filed April 21, 1951, now Patent No. 2,658,839, granted November 10, 1953, wherein the plating bath is recirculated between a plating chamber and a reservoir with the build-up of phosphite anions therein to a concentration in excess of one molar, without the precipitation of nickel phosphite and mixed basic salts.

In fact these plating baths exhibit normal plating rates in excess of 1 mil (0.001") per hour at optimum pH, above about 5.5, the higher pH favorably influencing the plating rate.

However, it has now been discovered that the chemical nickel plating process disclosed in the Gutzeit, Talmey and Lee application, when these plating baths of the higher pH are employed, is productive of nickel coatings

## 2

upon bodies formed essentially of iron, i. e., steel, etc., that are not quite as adherent as is desirable, particularly when the plated bodies are subjected to repeated strains in their subsequent use.

Also, it has been discovered that the resistance of these nickel coatings to electrolytic corrosion, as exhibited by salt spray tests, is dependent upon the homogeneity of the surface of the body, as influenced by the preparation or pretreatment thereof preceding the chemical nickel plating operation; and more specifically, it has been discovered that the resistance to electrolytic corrosion is more or less directly proportional to the homogeneity of the surface of the body, the more nearly homogeneous the surface of the body, the higher the resistance of the subsequently produced nickel coating is to electrolytic corrosion.

Accordingly, it is a general object of the present invention to provide an improved process of chemical nickel plating of bodies formed essentially of iron, employing plating baths of the nickel cation-hypophosphite anion type, that is productive of very adherent nickel coatings and that also exhibit great resistance to electrolytic corrosion.

Another object of the invention is to provide an improved process of producing a nickel coating of substantial thickness upon the surface of a body formed essentially of iron, employing chemical nickel plating, wherein the nickel coating possesses great adhesion, exhibits great resistance to flaking incident to strains of the body, and possesses high corrosion resistance.

A further object of the invention is to provide an improved process of pretreating a body formed essentially of iron, before chemical nickel plating of the body, whereby the subsequent chemical nickel plating of the body is productive of a superior nickel coating thereon.

These and other objects and advantages of the invention pertain to the particular arrangement of the steps of the process, as will be understood from the foregoing and following description.

In accordance with the process of the present invention, the article or body to be nickel plated and formed essentially of iron, including the various alloys thereof, i. e. steel, etc., is first subjected to a composite pretreatment, the following having been found to be highly successful:

1. The body is subjected to a conventional vapor degreasing step.
2. The body is then subjected to a conventional alkaline cleaning step at a temperature of about 180° F. for a time interval of about 5 to 20 minutes.
3. The body is then subjected to a rinsing step in water at a temperature of about 110° F. for a time interval of about 5 minutes.
4. The body is then subjected to a pickling step in an aqueous solution of hydrochloric acid at room temperature (about 70° F.) for a time interval of about 4 minutes, the solution containing about 15% HCl by weight.
5. The body is subjected to a repetition of step No. 3 above.
6. The body is subjected to a repetition of step No. 2 above.
7. The body is subjected to a repetition of step No. 3 above.
8. The body is subjected to a repetition of step No. 4 above.
9. The body is then subjected to a rinsing or soaking step in an aqueous solution of hydrogen peroxide at a temperature of about 110° F. for a time interval of about 5 minutes, the solution containing not in excess of about 0.1% of hydrogen peroxide by weight.

In this composite pretreatment, inclusion of steps Nos. 5 to 8, inclusive, set forth above, being repetitious of certain of the preceding steps, is optional, but preferably these steps are included as a matter of precaution, so as positively to insure that the surface of the body is in readiness to receive the very thin iron oxide film thereon, resulting from step No. 9, set forth above. Accordingly, this composite pretreatment positively insures cleaning and degreasing of the surface of the body, as well as the formation of the very thin iron oxide film thereon, without the formation of any visible rust thereon; whereby the surface of the body is made substantially homogeneous and lightly oxidized as noted above, the iron oxide film possibly being a film of  $Fe_3O_4$ . This homogeneity of the surface of the body brings about the subsequent production of a more homogeneous nickel coating thereon, thus preventing local galvanic action and electrochemical corrosion of the nickel coating and improving the corrosion resistance of the nickel coating to salt spray tests.

After the body has been subjected to the composite pretreatment described above, it is immersed in a hot strike bath consisting essentially of an aqueous solution of a nickel salt, and having a temperature slightly below the boiling point thereof, about 210° F., and having a pH in the approximate range of 1.9 to 3.5. More particularly, the body is immersed in the strike solution for a first time interval in excess of 3 minutes, up to about 10 minutes, that is sufficiently long to effect a displacement reaction resulting in the deposit of a thin nickel film upon the surface of the body in accordance with the equation:



This displacement reaction (1) proceeds only until the surface of the body is coated with a thin layer of nickel, and is substantially of monomolecular thickness; and preferably, the strike bath has a pH within the range 2.2 to 3.0.

After the body has been subjected to the nickel strike bath described above, it is immersed in a hot plating bath consisting essentially of an aqueous solution of a nickel salt and a hypophosphite, and having a temperature slightly below the boiling point thereof, about 210° F., and having a pH above 4.0. More particularly, the body is immersed in the plating bath for a second time interval sufficiently long to effect catalytic plating of additional nickel upon the thin nickel film previously mentioned and build-up of a composite nickel coating of substantial thickness upon the surface of the body in accordance with the overall equation:



This catalytic reaction (2) proceeds upon an autocatalytic basis so that the composite nickel coating upon the surface of the body may be built up to the desired thickness.

After the body has been subjected to the nickel plating bath described above, it is rinsed and is ready for use, the nickel coating thereon being firmly adhered thereto and exhibiting great resistance to flaking, particularly when the plated body is subjected to repeated strains in its subsequent use.

In passing, it is noted that there exist several methods for determining, in a more or less qualitative manner, the adhesion of a nickel coating or plating on a base metal; and specifically it has been found that a very satisfactory and simple procedure resides in: first providing an elongated steel strap having a thickness of about  $\frac{1}{4}$ " and a width of about  $\frac{3}{4}$ " to  $1\frac{1}{4}$ ", the midportion of the strap being necked down about  $\frac{1}{16}$ " along each edge thereof for a distance of at least 2"; then plating the steel strap in the manner previously described; then subjecting the plated steel strap to a tension breaking test; and then examining the raw broken edges of the two portions of the steel strap in order to determine the amount of flaking of the nickel coating adjacent to the break. Specifying

cally, it has been discovered that in the event no flaking of the nickel deposit occurs further back than  $\frac{1}{16}$ " from the break, the nickel coating possesses great adhesion and is not flaked by various other tests, including impact, compression, torsion, etc., tests. Accordingly, hereinafter in the testing of a sample in accordance with the procedure above-outlined: when the flaking of the nickel deposit back from the break is  $\frac{1}{16}$ ", the nickel coating is considered to be "good"; when the flaking of the nickel deposit back from the break is greater than  $\frac{1}{16}$ ", the nickel coating is considered to be "poor"; and when the flaking of the nickel deposit back from the break is less than  $\frac{1}{16}$ ", the nickel coating is considered to be "excellent". While it is appreciated that this standard is empirical, it is exceedingly useful, as a nickel coating that has been found to be "good" in accordance with this simple test, exhibits in other more complex tests great adhesion to the base metal.

In order to demonstrate the process of the present invention, an aqueous strike bath was prepared that had the following composition:

Strike bath SB1:

Nickel chloride \_\_\_\_\_ m. p. l. 0.0675  
Sodium succinate \_\_\_\_\_ m. p. l. 0.06  
pH adjusted with NaOH and HCl.

Also, an aqueous plating bath was prepared that had the following composition:

Plating bath PB1:

Malic acid \_\_\_\_\_ m. p. l. 0.135  
Aminoacetic acid \_\_\_\_\_ m. p. l. 0.0675  
Nickel chloride \_\_\_\_\_ m. p. l. 0.0675  
Sodium hypophosphite \_\_\_\_\_ m. p. l. 0.225  
2 p. p. m.  $Pb^{++}$  added as stabilizing ion.  
pH adjusted with NaOH and HCl.

Samples of cold rolled steel, each having an area of 80-85  $cm^2$ , were subjected to the composite pretreatment hereinbefore described, then rinsed in hot water, then immersed in the strike bath SB1 for a time interval of 3 minutes, and then immersed in the plating bath PB1 for an appropriate time interval. In this series of tests, the pH of the strike bath SB1 was varied, as indicated below; while the pH of the plating bath PB1 was established in the vicinity of 6.0, since this plating bath exhibits a plating rate greater than 1.1 mils per hour at this pH. The results of these tests were as follows:

| 50   | pH of Strike Bath SB1 | Initial pH of Plating Bath PB1 | Time of Plating (mins.) | Mils Plated | Adhesion   |
|------|-----------------------|--------------------------------|-------------------------|-------------|------------|
| 0.50 |                       | 6.20                           | 105                     | 3.76        | poor.      |
| 1.90 |                       | 6.20                           | 90                      | 3.20        | very good. |
| 2.30 |                       | 6.30                           | 155                     | 3.00        | Do.        |
| 2.40 |                       | 6.30                           | 170                     | 3.42        | Do.        |
| 4.00 |                       | 6.30                           | 110                     | 3.80        | fair.      |
| 4.60 |                       | 6.30                           | 110                     | 3.36        | poor.      |

The foregoing tests clearly demonstrate that in the present process, the pH of the strike bath SB1 should be in the approximate range 1.9 to 3.5, and preferably within the narrower range 2.2 to 3.0, in order to obtain maximum adhesion of the nickel coating upon the base metal sample.

In a number of subsequent tests, a number of other aqueous strike baths were prepared that had the compositions indicated below:

Strike bath SB2:

Nickel hypophosphite \_\_\_\_\_ m. p. l. 0.0675

Strike bath SB3:

Nickel chloride \_\_\_\_\_ m. p. l. 0.09

Strike bath SB4:

Nickel chloride \_\_\_\_\_ m. p. l. 0.0675

Sodium succinate \_\_\_\_\_ m. p. l. 0.06

## Strike bath SB5:

|                 |          |        |
|-----------------|----------|--------|
| Nickel chloride | m. p. l. | 0.0675 |
| Acetic acid     | m. p. l. | 0.06   |

## Strike bath SB6:

|                 |          |        |
|-----------------|----------|--------|
| Nickel chloride | m. p. l. | 0.0675 |
| Lactic acid     | m. p. l. | 0.06   |

## Strike bath SB7:

|                  |          |        |
|------------------|----------|--------|
| Nickel chloride  | m. p. l. | 0.0675 |
| Sodium succinate | m. p. l. | 0.06   |
| Sodium fluoride  | m. p. l. | 0.05   |

## Strike bath SB8:

|                  |          |        |
|------------------|----------|--------|
| Nickel chloride  | m. p. l. | 0.0675 |
| Aminoacetic acid | m. p. l. | 0.0675 |

## Strike bath SB9:

|                      |          |        |
|----------------------|----------|--------|
| Nickel hypophosphite | m. p. l. | 0.06   |
| Malic acid           | m. p. l. | 0.135  |
| Aminoacetic acid     | m. p. l. | 0.0675 |

## Strike bath SB10:

|                  |          |        |
|------------------|----------|--------|
| Nickel chloride  | m. p. l. | 0.0675 |
| Sodium succinate | m. p. l. | 0.06   |
| Malic acid       | m. p. l. | 0.06   |
| Lactic acid      | m. p. l. | 0.2025 |

## Plating bath PB6:

|                                  |          |        |
|----------------------------------|----------|--------|
| Nickel chloride                  | m. p. l. | 0.0675 |
| Sodium hypophosphite             | m. p. l. | 0.225  |
| Sodium succinate                 | m. p. l. | 0.12   |
| Malic acid                       | m. p. l. | 0.06   |
| Lactic acid                      | m. p. l. | 0.2025 |
| Pb <sup>++</sup> stabilizing ion | p. p. m. | 2      |

## Plating bath PB7:

|                                  |          |        |
|----------------------------------|----------|--------|
| Nickel chloride                  | m. p. l. | 0.0675 |
| Sodium hypophosphite             | m. p. l. | 0.225  |
| Malic acid                       | m. p. l. | 0.0675 |
| Aminoacetic acid                 | m. p. l. | 0.0675 |
| Pb <sup>++</sup> stabilizing ion | p. p. m. | 2      |

Additional samples of cold rolled steel, each having an area of 80-85 cm.<sup>2</sup>, were subjected to the composite pretreatment hereinbefore described; then rinsed in hot water; then immersed in one of the strike baths SB2 to SB12 for a time interval of 3 minutes, and then immersed in one of the plating baths PB2 to PB7, for an appropriate time interval. In this series of tests, the pH of the various strike baths were varied, as indicated below; while the pH of the various plating baths were selected substantially at the highest plating rate thereof. Illustrative results of this series of tests were as follows:

| Strike Bath No. | pH of Strike Bath | Plating Bath No. | Initial pH of Plating Bath | Time of Strike (Min.) | Time of Plating (Min.) | Mils Plated | Adhesion   |
|-----------------|-------------------|------------------|----------------------------|-----------------------|------------------------|-------------|------------|
| SB8             | 2.30              | PB2              | 5.60                       | 3                     | 110                    | 2.89        | good.      |
| SB8             | 2.30              | PB2              | 5.60                       | 4                     | 135                    | 3.19        | very good. |
| SB8             | 2.30              | PB2              | 5.60                       | 5                     | 115                    | 1.89        | excellent. |
| SB8             | 2.30              | PB2              | 5.60                       | 5                     | 115                    | 1.94        | Do.        |
| SB9             | 2.25              | PB3              | 5.70                       | 5                     | 108                    | 2.01        | very good. |
| SB4             | 2.15              | PB3              | 5.70                       | 3                     | 120                    | 2.05        | fair.      |
| SB7             | 2.30              | PB3              | 6.30                       | 5                     | 115                    | 2.71        | very good. |
| SB7             | 2.30              | PB3              | 6.00                       | 5                     | 65                     | 1.95        | Do.        |
| SB2             | 0.50              | PB2              | 5.50                       | 2                     | 115                    | 1.85        | poor.      |
| SB2             | 3.0               | PB3              | 5.50                       | 2                     | 140                    | 2.41        | good.      |

## Strike bath SB11:

|                  |          |        |
|------------------|----------|--------|
| Nickel chloride  | m. p. l. | 0.0675 |
| Sodium succinate | m. p. l. | 0.12   |
| Malic acid       | m. p. l. | 0.06   |

These plating tests again illustrate that the pH of the strike bath should be in the approximate range 1.9 to 3.5, and further demonstrate that the time of nickel strike is considerably reduced in the strike baths that also contain certain of the organic additives.

In a modified form of the present process, the body formed essentially of iron, after being subjected to the pretreatment previously described, is immersed in a hot bath of the plating type described, but having a relatively low pH of a value of around 4.5, for a time interval of 10 to 20 minutes; then the pH of the plating bath is increased stepwise to a value above about 5.5 by the corresponding additions thereto of a soluble alkali, such as caustic soda; and then the plating is continued at the relatively high pH for the required time interval to obtain the desired thickness of the nickel coating.

In order to demonstrate this modification of the present process a cold rolled steel sample of 80 cm.<sup>2</sup> area was first subjected to the composite pretreatment previously described; and a plating bath of 6 liters was prepared that had the following composition:

|                                  |          |        |
|----------------------------------|----------|--------|
| Nickel chloride                  | m. p. l. | 0.0675 |
| Sodium hypophosphite             | m. p. l. | 0.225  |
| Malic acid                       | m. p. l. | 0.2025 |
| Aminoacetic acid                 | m. p. l. | 0.0675 |
| Pb <sup>++</sup> stabilizing ion | p. p. m. | 2      |

This plating bath was divided into three equal parts of 2 liters each, and the pH was adjusted with NaOH and HCl as follows:

- Part 1—2 liters @ 4.50 pH
- Part 2—2 liters @ 5.20 pH
- Part 3—2 liters @ 6.20 pH

The previously prepared steel sample was placed in the plating chamber of the continuous plating system of the character disclosed in the previously mentioned Talmy and Crehan application; and then the first, second and third portions of this plating bath were suc-

## Strike bath SB12:

|                  |          |        |
|------------------|----------|--------|
| Nickel chloride  | m. p. l. | 0.0675 |
| Malic acid       | m. p. l. | 0.135  |
| Aminoacetic acid | m. p. l. | 0.0675 |

Also, a number of other aqueous plating baths were prepared that had the compositions indicated below:

## Plating bath PB2:

|                                  |          |        |
|----------------------------------|----------|--------|
| Nickel chloride                  | m. p. l. | 0.0675 |
| Sodium hypophosphite             | m. p. l. | 0.225  |
| Sodium succinate                 | m. p. l. | 0.06   |
| Malic acid                       | m. p. l. | 0.2025 |
| Pb <sup>++</sup> stabilizing ion | p. p. m. | 2      |

50

## Plating Bath PB3:

|                                  |          |        |
|----------------------------------|----------|--------|
| Nickel chloride                  | m. p. l. | 0.0675 |
| Sodium hypophosphite             | m. p. l. | 0.225  |
| Malic acid                       | m. p. l. | 0.2025 |
| Aminoacetic acid                 | m. p. l. | 0.0675 |
| Pb <sup>++</sup> stabilizing ion | p. p. m. | 2      |

55

## Plating bath PB4:

|                                  |          |        |
|----------------------------------|----------|--------|
| Nickel chloride                  | m. p. l. | 0.0675 |
| Sodium hypophosphite             | m. p. l. | 0.225  |
| Sodium succinate                 | m. p. l. | 0.20   |
| Malic acid                       | m. p. l. | 0.06   |
| Lactic acid                      | m. p. l. | 0.2025 |
| Pb <sup>++</sup> stabilizing ion | p. p. m. | 2      |

65

## Plating bath PB5:

|                                  |          |        |
|----------------------------------|----------|--------|
| Nickel chloride                  | m. p. l. | 0.0675 |
| Sodium hypophosphite             | m. p. l. | 0.225  |
| Sodium succinate                 | m. p. l. | 0.16   |
| Malic acid                       | m. p. l. | 0.06   |
| Lactic acid                      | m. p. l. | 0.2025 |
| Pb <sup>++</sup> stabilizing ion | p. p. m. | 2      |

75

cessively flowed through the plating chamber at a temperature of about 210° F., during a total time interval of 120 minutes. The weight gain of this steel sample was 3.7 grams; the nickel deposit had a thickness of 2.1 mils; and the adhesion of the nickel coating was excellent.

In passing, it is noted that in this modification of the present process, it is important to raise the pH of the plating bath gradually in order to obtain good adhesion of the nickel coating upon the base metal formed essentially of iron.

In another modified form of the present process, substantially identical to that described above, the body formed essentially of iron, after being subjected to the composite pretreatment previously described, is immersed in a hot bath of the strike type described consisting essentially of an aqueous acid solution of a nickel salt; and after the nickel strike upon the surface of the body, the strike bath is converted into a bath of the plating type described stepwise by the corresponding additions thereto of both a soluble hypophosphite and a soluble alkali, such as sodium hypophosphite and caustic soda; and in this modification of the present process, it is immaterial whether the various soluble organic additives are initially placed in the strike bath or are added thereto incident to the conversion of the strike bath into the plating bath.

In a further modified form of the present process, the body formed essentially of iron, is first subjected to the composite pretreatment previously described, and is then immersed in a cool bath of the plating type described at a temperature in the approximate range 130° F. to 150° F. for a time interval of about 10 to 20 minutes; and then the temperature of the plating bath is increased gradually to a temperature slightly below the boiling point thereof, about 210° F. In this modification of the present process, the initial nickel strike upon the surface of the body takes place very slowly in the relatively cool plating bath; and thereafter, the catalytic nickel plating and build-up of the nickel coating take place as time proceeds in the relatively hot plating bath.

In the formation of aqueous plating baths of the type disclosed in the Gutzeit, Talmey and Lee application mentioned, the soluble nickel salt may take a variety of forms, such, for example, as nickel chloride, nickel sulfate, etc., or mixtures thereof; and the soluble hypophosphite may take a variety of forms, such, for example, as sodium hypophosphite, potassium hypophosphite, calcium hypophosphite, etc., or mixtures thereof. In the plating bath, the absolute concentration of hypophosphite ions is in the approximate range 0.15 to 1.20 mole/liter, and the ratio between nickel ions and hypophosphite ions is in the approximate range 0.25 to 1.60.

A typical malic acid-lactic acid-succinate plating bath of this type further comprises an absolute concentration of malic acid ions in the approximate range 0.04 to 0.20 mole/liter; an absolute concentration of lactic acid ions in the approximate range 0.04 to 0.20 mole/liter; the total quantity of the malic acid ions and the lactic acid ions are sufficient to complex at least 100% of the nickel ions; an absolute concentration of succinic acid ions of at least 0.04 mole/liter; and a pH within the approximate range 4.5 to 7.0.

A typical malic acid-glycine plating bath of this type further comprises an absolute concentration of malic acid ions sufficient to complex at least 100% of the nickel ions; an absolute concentration of glycine ions of at least 0.04 mole/liter; and a pH within the approximate range 4.5 to 9.5.

A typical malic acid-succinate plating bath of this type further comprises an absolute concentration of malic acid ions sufficient to complex at least 100% of the nickel ions; an absolute concentration of succinic acid ions of at least 0.04 mole/liter; and a pH within the approximate range 4.5 to 7.0.

These plating baths of the type described are particularly well suited for use in a continuous plating system

of the character noted, as they exhibit a fast plating rate, have an exceedingly long life, and maintain nickel phosphite in solution in concentrations as high as one molar. Moreover, when these plating baths are employed in the present process, the nickel coatings upon bodies formed essentially of iron, including the various alloys thereof, i. e. steel, etc., are exceedingly adherent, homogeneous, smooth and bright.

In view of the foregoing, it is apparent that there has been provided an improved process of chemical nickel plating of bodies formed essentially of iron, including the various alloys thereof, i. e. steel, etc., that is productive of exceedingly adherent nickel coatings having high resistance to electrolytic corrosion whereby the process is particularly well suited to the chemical nickel plating of forged and cast steel elements and parts.

While there has been described what is at present considered to be the preferred embodiment of the invention, it will be understood that various modifications may be made therein, and it is intended to cover in the appended claims all such modifications as fall within the true spirit and scope of the invention.

What is claimed is:

1. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface of said body and without the formation of any visible rust upon the surface thereof, said solution containing not in excess of about 0.1% by weight of hydrogen peroxide, then contacting said body with a first hot nickel plating bath comprising an aqueous solution of a nickel salt and having a temperature slightly below the boiling point thereof and having a pH in the approximate range 1.9 to 3.5 during a first time interval sufficiently long to effect the displacement deposit of a thin nickel film upon the surface of said body, and then contacting said body with a second hot nickel plating bath comprising an aqueous solution of a nickel salt and a hypophosphite and having a temperature slightly below the boiling point thereof and having a pH in the approximate range 4.0 to 9.5 during a second time interval sufficiently long to effect the catalytic plating of additional nickel upon said thin nickel film and the build-up of a composite nickel coating of substantial thickness upon the surface of said body.
2. The process of producing a nickel coating of substantial thickness upon the surface of a body formed essentially of iron, which comprises cleaning and degreasing the surface of said body, rinsing the surface of said body in an aqueous solution of hydrogen peroxide to form a thin iron oxide film upon the surface thereof and without the formation of any visible rust upon the surface thereof, said solution containing not in excess of about 0.1% by weight of hydrogen peroxide, then contacting said body with a first hot nickel plating bath comprising an aqueous solution of a nickel salt and having a temperature slightly below the boiling point thereof and having a pH in the approximate range 1.9 to 3.5 during a first time interval sufficiently long to effect the displacement deposit of a thin nickel film upon the surface of said body, and then contacting said body with a second hot nickel plating bath comprising an aqueous solution of a nickel salt and a hypophosphite and having a temperature slightly below the boiling point thereof and having a pH in the approximate range 4.0 to 9.5 during a second time interval sufficiently long to effect the catalytic plating of additional nickel upon said thin nickel film and the build-up of a composite nickel coating of substantial thickness upon the surface of said body.
3. The process of plating with nickel the surface of a body formed essentially of iron, which comprises cleaning and degreasing the surface of said body, contacting said body with an aqueous solution of hydrogen peroxide

for a time interval sufficiently long to form only a thin iron oxide film upon the surface of said body and without the formation of any visible rust upon the surface thereof, said solution containing not in excess of about 0.1% by weight of hydrogen peroxide, and then contacting said body with a nickel plating bath comprising an aqueous acid solution of a nickel salt and having a pH in the approximate range 2.2 to 3.0 in order to effect the displacement deposit of a thin nickel film upon the surface of said body.

4. The process of plating with nickel the surface of a body formed essentially of iron, which comprises cleaning and degreasing the surface of said body, soaking said body in an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, and then contacting said body with a nickel plating bath of an aqueous solution of a nickel salt in order to effect the displacement deposit of a thin nickel film upon the surface of said body.

5. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, contacting said body with a first nickel plating bath comprising an aqueous solution of a nickel salt and having a pH in the approximate range 1.9 to 3.5 during a first time interval sufficiently long to effect the displacement deposit of a thin nickel film upon the surface of said body, and then contacting said body with a second nickel plating bath comprising an aqueous solution of a nickel salt and a hypophosphite and having a pH in the approximate range 4.0 to 9.5 during a second time interval sufficiently long to effect the catalytic plating of additional nickel upon said thin nickel film and build-up of a composite nickel coating of substantial thickness upon the surface of said body.

6. The process set forth in claim 5, wherein said first and second nickel plating baths have temperatures slightly below the boiling points thereof and said first time interval is in the approximate range 3 to 10 minutes and said second time interval is at least 60 minutes.

7. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface of said body and without the formation of any visible rust upon the surface thereof, said solution containing not in excess of 0.1% by weight of hydrogen peroxide, contacting said body with a first nickel plating bath comprising an aqueous solution of a nickel salt and having a pH in the approximate range 2.2 to 3.0 during a first time interval sufficiently long to effect the displacement deposit of a thin nickel film upon the surface of said body, and then contacting said body with a second nickel plating bath comprising an aqueous solution of a nickel salt and a hypophosphite and having a pH in the approximate range 4.0 to 9.5 during a second time interval sufficiently long to effect the catalytic plating of additional nickel upon said thin nickel film and the build-up of a complete nickel coating of substantial thickness upon the surface of said body.

8. The process of producing a nickel coating of substantial thickness upon the surface of a body formed essentially of iron, which comprises cleaning and degreasing the surface of said body with an aqueous solution of hy-

drogen peroxide for a time interval sufficiently long to form only a thin iron oxide film upon the surface thereof and without the formation of any visible rust upon the surface thereof, said solution containing not in excess of about 1.0% by weight of hydrogen peroxide, contacting said body with a first nickel plating bath comprising an aqueous solution of a nickel salt and also containing an additive selected from the group consisting of short chain saturated aliphatic carboxylic acids and alkaline salts there-

of and having a pH in the approximate range 1.9 to 3.5 during a first time interval sufficiently long to effect the displacement deposit of a thin nickel film upon the surface of said body, and then contacting said body with a second nickel plating bath comprising an aqueous solution of a nickel salt and a hypophosphite and also containing an additive selected from the group consisting of short chain saturated aliphatic carboxylic acids and alkaline salts there-

of and having a pH in the approximate range 5.5 to 9.5 during a second time interval sufficiently long to effect the catalytic plating of additional nickel upon said thin nickel film and the build-up of a composite nickel coating of substantial thickness upon the surface of said body.

9. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, providing a first nickel plating bath comprising an aqueous solution of a nickel salt and having a pH in the approximate range 1.9 to 3.5, providing a second nickel plating bath comprising an aqueous solution of a nickel salt and a hypophosphite and having a pH in the approximate range 4.0 to 9.5 immersing said body in said first nickel plating bath to effect the displacement deposit of a thin nickel film upon the surface thereof, withdrawing said body from said first nickel plating bath and immersing it in the said second nickel plating bath to effect the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

10. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, providing a first nickel plating bath comprising an aqueous solution of a nickel salt and having a pH in the approximate range 1.9 to 3.5, providing a second nickel plating bath comprising an aqueous solution of a nickel salt and a hypophosphite and having a pH in the approximate range 4.0 to 9.5 immersing said body in said first nickel plating bath to initiate the displacement deposit of nickel upon the surface thereof, withdrawing said body from said first nickel plating bath after a time interval sufficiently long to effect the displacement plating of a thin nickel film upon the surface thereof, immersing said body in said second nickel plating bath to initiate the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

75

11. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, providing a first nickel plating bath comprising an aqueous solution of a nickel salt and having a pH in the approximate range 1.9 to 3.5, immersing said body in said first nickel plating bath to initiate the displacement deposit of nickel upon the surface thereof, converting said first nickel plating bath into a second nickel plating bath after a time interval sufficiently long to effect the displacement deposit of a thin nickel film upon the surface of said body by the addition to said first nickel plating bath of both a soluble hypophosphite and a soluble alkali so that the pH of said second nickel plating bath is brought up into the approximate range 4.0 to 9.5 in order to initiate the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

12. The process set forth in claim 11, wherein said conversion of said first nickel plating bath into said second nickel plating bath is made in a number of steps by the additions at a corresponding number of spaced time intervals of appropriate small quantities of said soluble hypophosphite and said soluble alkali to said first nickel plating bath.

13. The process of producing a nickel coating of substantial thickness upon the surface of a body formed essentially of iron, which comprises cleaning and degreasing the surface of said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, providing a first nickel plating bath comprising an aqueous solution of a nickel salt and also containing an additive selected from the group consisting of short chain saturated aliphatic carboxylic acids and alkaline salts thereof and having a pH in the approximate range 1.9 to 3.5, immersing said body in said first nickel plating bath to initiate the displacement deposit of nickel upon the surface thereof, converting said first nickel plating bath into a second nickel plating bath after a time interval sufficiently long to effect the displacement deposit of a thin nickel film upon the surface of said body by the addition to said first nickel plating bath of both a soluble hypophosphite and a soluble alkali so that the pH of said second nickel plating bath is brought up into the approximate range 4.0 to 9.5 in order to initiate the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

14. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of about 0.1% by weight of hydrogen peroxide, providing a first nickel plating bath comprising an aqueous solution of a nickel salt and a

hypophosphite and having a pH in the approximate range 1.9 to 3.5, immersing said body in said first nickel plating bath to initiate the displacement deposit of nickel upon the surface thereof, converting said first nickel plating bath into a second nickel plating bath after a time interval sufficiently long to effect the displacement deposit of a thin nickel film upon the surface of said body by the addition to said first nickel plating bath of a soluble alkali so that the pH of said second nickel plating bath is brought up into the approximate range 4.0 to 9.5 in order to effect the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

15. The process set forth in claim 14, wherein said conversion of said first nickel plating bath into said second nickel plating bath is made in a number of steps by the additions at a corresponding number of spaced time intervals of appropriate small quantities of said soluble alkali to said first nickel plating bath.

16. The process of producing a nickel coating of substantial thickness upon the surface of a body formed essentially of iron, which comprises cleaning and degreasing the surface of said body, contacting said body with an aqueous solution of hydrogen peroxide for a time interval sufficiently long to form only a thin iron oxide film upon the surface thereof and without the formation of any visible rust upon the surface thereof, said solution containing not in excess of 0.1% by weight of hydrogen peroxide, providing a first nickel plating bath comprising an aqueous solution of a nickel salt and a hypophosphite and also containing an additive selected from the group consisting of short chain saturated aliphatic carboxylic acids and alkaline salts thereof and having a pH in the approximate range 1.9 to 3.5, immersing said body in said first nickel plating bath to initiate the displacement deposit of nickel upon the surface thereof, converting said first nickel plating bath into a second nickel plating bath after a time interval sufficiently long to effect the displacement deposit of a thin nickel film upon the surface of said body by the addition to said first nickel plating bath of a soluble alkali so that the pH of said second nickel plating bath is brought up into the approximate range 4.0 to 9.5 in order to effect the catalytic plating of additional nickel upon said thin nickel film and the build-up of a composite nickel coating upon the surface of said body, and withdrawing said body from said second nickel plating bath when the composite nickel coating upon the surface thereof has reached the substantial thickness desired.

17. The process of producing a nickel coating of substantial thickness upon the surface of a body formed essentially of iron, which comprises cleaning and degreasing the surface of said body, rinsing the surface of said body in an aqueous solution of hydrogen peroxide to form a thin iron oxide film upon the surface thereof and without the formation of any visible rust upon the surface thereof, said solution containing not in excess of about 0.1% by weight of hydrogen peroxide, providing a nickel plating bath comprising an aqueous solution of a nickel salt and a hypophosphite and having a temperature slightly below the boiling point thereof, and immersing said body in said nickel plating bath during a time interval sufficiently long to effect plating of a nickel coating of substantial thickness upon the surface of said body.

18. The process set forth in claim 17, wherein said nickel plating bath has a pH in the approximate range 5.5 to 9.5.

19. The process of producing a nickel coating of substantial thickness upon the surface of a body formed essentially of iron, which comprises cleaning and degreasing of the surface of said body, forming a thin iron oxide film upon the surface of said body and without the for-

mation of any visible rust upon the surface thereof by soaking said body in a warm aqueous solution of hydrogen peroxide, said solution having a temperature of about 110° F. and containing not in excess of about 0.1% by weight of hydrogen peroxide, providing a nickel plating bath comprising an aqueous solution of a nickel salt and a hypophosphite and also containing an additive selected from the group consisting of short chain saturated aliphatic carboxylic acids and alkaline salts thereof and having a pH in the approximate range 5.5 to 9.5, and immersing said body in said nickel plating bath during a time interval sufficiently long to effect plating of a nickel coating of substantial thickness upon the surface of said body.

20. The process of producing a nickel coating of substantial thickness upon the surface of a body formed essentially of iron, which comprises cleaning and degreasing the surface of said body, forming a thin iron oxide film upon the surface of said body and without the formation of any visible rust upon the surface thereof by soaking said body in an aqueous solution of hydrogen peroxide, said solution containing not in excess of about 0.1% by weight of hydrogen peroxide, immersing said body in a cool nickel plating bath comprising an aqueous solution of a nickel salt and a hypophosphite, said nickel plating bath having a temperature well below the boiling point thereof, increasing the temperature of said nickel plating bath to a temperature slightly below the boiling point thereof, and withdrawing said body from said hot nickel plating bath after a time interval sufficiently long to effect plating of a nickel coating of substantial thickness upon the surface of said body.

21. The process of producing a nickel plating of substantial thickness upon the surface of a body formed

5 essentially of iron, which comprises cleaning and degreasing the surface of said body, forming a thin iron oxide film upon the surface of said body and without the formation of any visible rust upon the surface thereof by soaking said body in an aqueous solution of hydrogen peroxide, said solution containing not in excess of about 0.1% by weight of hydrogen peroxide, providing a cool nickel plating bath comprising an aqueous solution of a nickel salt and a hypophosphite and also containing an additive selected from the group consisting of short chain saturated aliphatic carboxylic acids and alkaline salts thereof and having a pH in the approximate range 5.5 to 9.5, said nickel plating bath having a temperature well above the boiling point thereof, immersing said body in said cool nickel plating bath, increasing the temperature of said nickel plating bath to a temperature slightly below the boiling point thereof, and withdrawing said body from said hot nickel plating bath after a time interval sufficiently long to effect plating of a nickel coating of substantial thickness upon the surface of said body.

References Cited in the file of this patent

UNITED STATES PATENTS

|    |           |                |               |
|----|-----------|----------------|---------------|
| 25 | 24,604    | Pomeroy        | June 28, 1859 |
|    | 1,207,218 | Roux           | Dec. 5, 1916  |
|    | 1,383,703 | Elmen          | July 5, 1921  |
|    | 2,387,335 | Leonard        | Oct. 23, 1945 |
|    | 2,532,283 | Brenner et al. | Dec. 5, 1950  |
| 30 | 2,581,310 | Sweo           | Jan. 1, 1952  |
|    | 2,658,842 | Gutzeit et al. | Nov. 10, 1953 |

FOREIGN PATENTS

|         |               |               |
|---------|---------------|---------------|
| 385,582 | Great Britain | Mar. 23, 1931 |
|---------|---------------|---------------|